



US009316936B2

(12) **United States Patent**  
**Marcell et al.**

(10) **Patent No.:** **US 9,316,936 B2**  
(45) **Date of Patent:** **Apr. 19, 2016**

(54) **COLORED TONERS**

(71) Applicant: **Xerox Corporation**, Norwalk, NY (US)

(72) Inventors: **Kevin F Marcell**, Webster, NY (US);  
**Maria M Barden**, Fairport, NY (US);  
**Kimberly Anne Stoll**, Penfield, NY  
(US); **Christopher M Wolfe**, Rochester,  
NY (US); **Brian J Andaya**, Ontario, NY  
(US)

(73) Assignee: **Xerox Corporation**, Norwalk, CT (US)

(\*) Notice: Subject to any disclaimer, the term of this  
patent is extended or adjusted under 35  
U.S.C. 154(b) by 0 days.

(21) Appl. No.: **14/012,007**

(22) Filed: **Aug. 28, 2013**

(65) **Prior Publication Data**

US 2015/0072283 A1 Mar. 12, 2015

(51) **Int. Cl.**

**G03G 9/09** (2006.01)  
**G03G 9/08** (2006.01)  
**G03G 9/087** (2006.01)  
**G03G 9/093** (2006.01)  
**G03G 9/097** (2006.01)

(52) **U.S. Cl.**

CPC ..... **G03G 9/0804** (2013.01); **G03G 9/0819**  
(2013.01); **G03G 9/0821** (2013.01); **G03G  
9/08755** (2013.01); **G03G 9/08782** (2013.01);  
**G03G 9/08797** (2013.01); **G03G 9/09**

(2013.01); **G03G 9/09328** (2013.01); **G03G  
9/09708** (2013.01); **G03G 9/09725** (2013.01);  
**Y10T 428/2982** (2015.01)

(58) **Field of Classification Search**

CPC ... G03G 9/09; G03G 9/0918; G03G 9/08755;  
G03G 9/08797; G03G 9/092; G03G 9/0819  
USPC ..... 430/107.1, 108.1  
See application file for complete search history.

(56) **References Cited**

U.S. PATENT DOCUMENTS

6,028,178 A \* 2/2000 Metz et al. ..... 534/581  
6,635,398 B1 \* 10/2003 Komoto et al. ..... 430/108.23  
6,784,231 B2 \* 8/2004 Shimada ..... C09B 67/0015  
106/447  
2003/0110982 A1 \* 6/2003 Shimada et al. ..... 106/496  
2006/0154162 A1 \* 7/2006 Zhou ..... G03G 9/0804  
430/108.1  
2006/0172212 A1 \* 8/2006 Step et al. ..... 430/108.4  
2007/0003856 A1 \* 1/2007 Farrugia et al. ..... 430/110.2  
2007/0169666 A1 \* 7/2007 Brychcy et al. ..... 106/31.78  
2007/0254228 A1 \* 11/2007 Farrugia ..... G03G 9/09741  
430/108.2  
2011/0008720 A1 \* 1/2011 Yasukawa et al. ..... 430/107.1

\* cited by examiner

Primary Examiner — Hoa V Le

(74) Attorney, Agent, or Firm — Marylou J. Lavoie, Esq.  
LLC

(57) **ABSTRACT**

The disclosure describes a pigment of certain surface area for  
use in toner.

**20 Claims, No Drawings**

**1**  
**COLORED TONERS**

**FIELD**

Toners made with pigment particles of certain BET surface area; developers comprising said toners; devices comprising said toners and developers; imaging device components comprising said toners and developers; imaging devices comprising said developers; and so on, are described.

**BACKGROUND**

Some pigments and colored toner components have electronic properties that may confound or diminish efficacy of a toner containing same. For example, carbon black has high color density (coloring per unit weight), high blackness degree and high light fatness. However, higher levels of black pigment in a toner can result in lower charging with higher dielectric loss, both of which reduce transfer efficiency and degrade image quality (IQ). Black pigments are known to be more conductive than other pigments, which may be due to the formation of conductive pathways by the pigment through the toner particle.

Therefore, there remains a need to enhance colored toner efficacy and thus, improve charging in the formulation of colored toner, for example, to enable robust use of some pigments in toners, to enable higher pigment loading in a toner and efficient color imaging.

**SUMMARY**

The instant disclosure describes toners comprising pigment particles comprising a BET surface area of from about 60 m<sup>2</sup>/g to about 95 m<sup>2</sup>/g, from about 70 m<sup>2</sup>/g to about 90 m<sup>2</sup>/g, from about 75 m<sup>2</sup>/g to about 85 m<sup>2</sup>/g. In embodiments, toner particles comprising said pigment of certain particle size comprise at least about 5.53 µm, at least about 5.55 µm, at least about 5.57 µm D<sub>50</sub> volume diameter. Such toner particles have improved electronic properties, such as J zone (70° F., 10% RH) charging, as compared to comparable toner comprising pigment particles of lesser BET surface area and in embodiments, of lesser size.

**DETAILED DESCRIPTION**

Pigments are insoluble colorants that can be isolated from natural sources or synthesized. Pigments generally are available as powders. Because pigments generally are insoluble in solvents, pigments form dispersions or suspensions. Optionally, surfactants, wetting agents, amphipathic compounds and so on can be included to facilitate dispersibility in solution.

Size of the toner and pigment particles can be obtained using materials and methods known in the art. Devices that can be used to obtain volume diameters of particles include MICROMERITICS Saturn DigiSizer, Beckman coulter MULTISIZER 3, Malvern Mastersizer and Zetasizer, Brookhaven 90Plus and NanoDLS and so on.

BET surface area of particles can be obtained using materials and methods known in the art. Devices that can be used to obtain BET surface area include Horiba SA-9600, MICROMERITICS ASAP 2020 Physisorption Analyzer, Quantachrome Instruments Monosorb and so on.

It was uncovered, unexpectedly that pigment particles of certain surface are enhance toner function. The pigment particles have a BET surface area of from about 60 m<sup>2</sup>/g to about 95 m<sup>2</sup>/g to about 9 m<sup>2</sup>/g from about 75 m<sup>2</sup>/g to about 85 m<sup>2</sup>/g. The toner particles comprising said pigment particles can

**2**

comprise a size of at least about 5.53 µm, at least about 5.55 µm, at least about 5.57 µm in D<sub>50</sub> volume diameter.

Unless otherwise indicated, all numbers expressing quantities are conditions, and so forth used in the specification and claims are to be understood as being modified in all instances by the term, "about." "About," is meant to indicate a variation of no more than 10% from the stated value. Also used herein is the term, "equivalent," "similar," "essentially," "substantially," "approximating" and "matching," or grammatical variations thereof, have generally acceptable definitions or at the least, are understood to have the same meaning as, "about." I. Toner Particles

Toner particles of interest can comprise a polyacrylate, a polystyrene, a polyester resin and so on, as known in the art. 15 A resin-forming monomer can be reacted with suitable other reactants to form a polymer resin.

Examples of suitable resins or polymers which may be utilized in forming a toner include, but are not limited to, poly(styrene-butadiene), poly(methylstyrene-butadiene), 20 poly(methyl methacrylate-butadiene), poly(ethyl methacrylate-butadiene), poly(propyl methacrylate-butadiene), poly(butyl methacrylate-butadiene), poly(methyl acrylate-butadiene), poly(styrene-isoprene), poly(methylstyrene-isoprene), poly(methyl methacrylate-isoprene), poly(ethyl methacrylate-isoprene), poly(propyl methacrylate-isoprene), poly(butyl methacrylate-isoprene), poly(methyl acrylate-isoprene), poly(ethyl acrylate-isoprene), poly(propyl acrylate-isoprene), poly(butyl acrylate-isoprene); poly(styrene-propyl acrylate), poly(styrene-butyl acrylate), poly(styrene-butadiene-acrylic acid), poly(styrene-butadiene-methacrylic acid), poly(styrene-butadiene-acrylonitrile-acrylic acid), poly(styrene-butyl acrylate-acrylic acid), poly(styrene-butyl acrylate-methacrylic acid), 30 poly(styrene-butyl acrylate-acrylonitrile), poly(styrene-butyl acrylate-acrylonitrile-acrylic acid), and combinations thereof.

A toner composition can comprise more than one form or sort of polymer, such as, two or more different polymers, such as, two or more different polyester polymers composed of 40 different monomers. The polymer can be an alternating copolymer, a block copolymer, a graft copolymer, a branched copolymer, a crosslinked copolymer and so on.

The toner particle can include other optional reagents, such as, a surfactant, a wax, a shell and so on. The toner composition 45 optionally can comprise inert particles, which can serve as toner particle carriers, which can comprise the resin taught herein. The inert particles can be modified, for example, to serve a particular function. Hence, the surface thereof can be derivatized or the particles can be manufactured for a desired purpose, for example, to carry a charge or to possess a magnetic field.

The toner particles comprise one or more pigments, wherein the pigment particles comprise a BET surface area of from about 60 m<sup>2</sup>/g to about 95 m<sup>2</sup>/g, from about 70 m<sup>2</sup>/g to 55 about 90 m<sup>2</sup>/g, from about 75 m<sup>2</sup>/g to about 85 m<sup>2</sup>/g. The toner particles comprising said pigment particles of certain BET surface area can be at least about 5.53 µm, at least about 5.55 µm, at least about 5.57 µm in D<sub>50</sub> volume diameter.

The discussion below is directed to polyester resins although any resin usable in a toner can be used.

A. Components

1. Resin

Toner particles of the instant disclosure include a resin-forming monomer suitable for use in forming a particulate containing or carrying one or more colorants of a toner for use in certain imaging devices, wherein at least one colorant comprises a pigment treated with a rosin product. The poly-

ester-forming monomer is one that is inducible to form a resin, that is, which reacts, sets or solidifies to form a solid. Such a resin, a plastic, an elastomer and so on, whether naturally occurring or synthetic, is one that can be used in an imaging device. Generally, any suitable monomer or monomers are induced to polymerize to form a polyester resin or copolymer. Any polyfunctional monomer may be used depending on the particular polyester polymer desired in a toner particle. Hence, bifunctional reagents, trifunctional reagents and so on can be used. One or more reagents that comprise at least three functional groups are incorporated into a polymer or into a branch to enable branching, further branching and/or crosslinking. Examples of such polyfunctional monomers include 1,2,4-benzene-tricarboxylic acid, 1,2,4-cyclohexanetricarboxylic acid, 2,5,7-naphthalenetricarboxylic acid, 1,2,4-naphthalenetricarboxylic acid, 1,2,5-hexanetricarboxylic acid, 1,3-dicarboxyl-2-methyl-2-methylene-carboxylpropane, tetra(methylene-carboxyl)methane and 1,2,7,8-octanetetracarboxylic acid. Polyester resins, for example, can be used for applications requiring low melting temperature. Formed particles can be mixed with other reagents, such as, a colorant, to form a developer.

One, two or more polymers may be used in forming a toner or toner particle. In embodiments where two or more polymers are used, the polymers may be in any suitable ration (e.g., weight ration) such as, for instance, with two different polymers, from about 1% (first polymer)/99% (second polymer) to about 99% (first polymer)/1% (second polymer), from about 10% (first polymer)/90% (second polymer) to about 90% (first polymer)/10% (second polymer) and so on, as a design choice. For example, a toner can comprise two forms of amorphous polyester resins and crystalline resin in relative amounts as a design choice.

The polymer may be present in an amount of from about 65 to about 95% by weight, from about 75 to about 85% by weight of toner particles on a solids basis.

#### a. Polyester Resins

Suitable polyester resins include, for example, those which are sulfonated, non-sulfonated, crystalline, amorphous, combinations thereof and the like. The polyester resins may be linear, branched, crosslinked, combinations thereof and the like. Polyester resins may include those described, for example, in U.S. Pat. Nos. 6,593,049; 6,830,860; 7,754,406; 7,781,138; 7,749,672; and 6,756,176, the disclosures of each of which hereby are incorporated by reference in entirety.

When a mixture is used, such as, amorphous and crystalline polyester resins, the ratio of crystalline polyester resin to amorphous polyester resin can be in the range from about 1:99 to about 50:50; from about 5:95 to about 40:60; from about 5:95 to about 35:65.

A polyester resin may be obtained synthetically, for example, in an esterification reaction involving a reagent comprising a carboxylic acid group and another reagent comprising an alcohol. In embodiments, the alcohol reagent comprises two or more hydroxyl groups, three or more hydroxyl groups. In embodiments, the acid comprises two or more carboxylic acid groups, three or more carboxylic acid groups. Reagents comprising three or more functional groups enable, promote or enable and promote polymer branching and crosslinking. In embodiments, a polymer backbone or a polymer branch comprises at least one monomer unit comprising at least one pendant group or side group, that is, the monomer reactant from which the unit was obtained comprises at least three functional groups.

Examples of polyacids or polyesters that can be used for preparing an amorphous polyester resin include terephthalic acid, phthalic acid, isophthalic acid, fumaric acid, trimellitic

acid, diethyl fumarate, dimethyl itaconate, cis-1,4-diacetoxy-2-butene, dimethyl fumarate, diethyl maleate, maleic acid, succinic acid, itaconic acid, succinic acid, cyclohexanoic acid, succinic anhydride, dodecylsuccinic acid, dodecylsuccinic anhydride, glutaric acid, glutaric anhydride, adipic acid, pimelic acid, suberic acid, azelaic acid, dodecanedioic acid, dimethyl naphthalenedicarboxylate, dimethyl terephthalate, diethyl terephthalate, dimethylisophthalate, diethylisophthalate, dimethylphthalate, phthalic anhydride, diethylphthalate, dimethylsuccinate, naphthalene dicarboxylic acid, dimer diacid, dimethylfumarate, dimethylmaleate, dimethylglutarate, dimethyladipate, dimethyl dodecylsuccinate, and combinations thereof. The polyacid or polyester reagent may be present, for example, in an amount from about 40 to about 60 mole % of the resin, from about 42 to about 52 mole % of the resin, from about 45 to about 50 mole % of the resin, and optionally a second polyacid can be used in an amount from about 0.1 to about 10 mole % of the resin.

Examples of polyols which may be used in generating an amorphous polyester resin include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, 1,4-cyclohexanediol, 1,3-cyclohexanediol, xylenedimethanol, cyclohexanediol, diethylene glycol, bis(2-hydroxyethyl) oxide, dipropylene glycol, dibutylene glycol, and combinations thereof. The amount of polyol can vary, and may be present, for example, in an amount from about 40 to about 60 mole % of the resin, from about 42 to about 55 mole % of the resin, from about 45 to about 53 mole % of the resin, and a second polyol, can be used in an amount from about 0.1 to about 10 mole %, from about 1 to about 4 mole % of the resin.

Polycondensation catalysts may be used in forming the amorphous (or crystalline) polyester resin, and include tetraalkyl titanes, dialkyltin oxides, such as, dibutyltin oxide, tetraalkyltins, such as, bibutyltin dilaurate, and dialkyltin oxide hydroxides, such as, butyltin oxide hydroxide, aluminum alkoxides, alkyl zinc, dialkyl zinc, zinc oxide, stannous oxide, or combinations thereof. Such catalysts may be used in an amount of, for example, from about 0.01 mole % to about 5 mole % based on the starting polyacid or polyester reagent(s) used to generate the polyester resin.

Examples of amorphous resins which may be used include alkali sulfonated-polyester resins, branched alkali sulfonated-polyester resins, alkali sulfonated-polyimide resins and branched alkali sulfonated-polyimide resins. Alkali sulfonated polyester resins may be useful in embodiments, such as, the metal or alkali salts of copoly(ethylene-terephthalate)-copoly(ethylene-5-sulfo-isophthalate), copoly(propylene-terephthalate)-copoly(propylene-5-sulfo-isophthalate), copoly(diethylene-terephthalate)-copoly(diethylene-5-sulfo-isophthalate), copoly(propylene-diethylene-terephthalate)-copoly(propylene-diethylene-5-sulfoisophthalate), copoly(propylene-butylene-terephthalate)-copoly(propylene-butylene-5-sulfo-isophthalate) and so on, wherein the alkali metal is, for example, a sodium, a lithium or a potassium ion.

In embodiments, an unsaturated amorphous polyester resin may be used as a latex resin. Examples of such resins include those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-male-

ate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate) and combinations thereof.

For forming a crystalline polyester resin, suitable polyols include aliphatic polyols with from about 2 to 36 carbon atoms, such as 1,2-ethanediol, 1,3-propanediol, 1,4-butanediol, 1,5-pentanediol, 2,2-dimethylpropane-1,3-diol, 1,6-hexanediol, 1,7-heptanediol, 1,8-octanediol, 1,9-nonanediol, 1,10-decanediol, 1,12-dodecanediol and the like; alkali sulfo-aliphatic diols such as sodio 2-sulfo-1,2-ethanediol, lithio 2-sulfo-1,2-ethanediol, potassium 2-sulfo-1,2-ethanediol, sodio 2-sulfo-1,3-propanediol, lithio 2-sulfo-1,3-propanediol, potassium 2-sulfo-1,3-propanediol, mixture thereof, and the like, including their structural isomers. The aliphatic polyol may be, for example, selected in an amount from about 40 to about 60 mole %, from about 42 to about 55 mole %, from about 45 to about 53 mole %, and optionally a second polyol, can be used in an amount from about 0.1 to about 10 mole %, from about 1 to about 4 mole % of the resin.

Examples of polyacid or polyester reagents for preparing a crystalline resin include oxalic acid, succinic acid, glutaric acid, adipic acid, suberic acid, azelaic acid, sebacic acid, fumaric acid, dimethyl fumarate, dimethyl itaconate, cis, 1,4-diacetoxy-2-butene, diethyl fumarate, diethyl maleate, phthalic acid, isophthalic acid, terephthalic acid, naphthalene-2,6-dicarboxylic dicarboxylic acid, naphthalene-2,7-dicarboxylic acid, cyclohexane dicarboxylic acid (sometimes referred to herein, in embodiments, as cyclohexanedioic acid), malonic acid and mesaconic acid, a polyester or anhydride thereof; and an alkali sulfo-organic polyacid, such as, the sodio, lithio or potassium salt of dimethyl-5-sulfo-isophthalate, dialkyl-5-sulfo-isophthalate-4-sulfo-1,8-naphthalic anhydride 4-sulfo-phthalic acid, dimethyl-4-sulfo-phthalate, dialkyl-4-sulfo-phthalate, 4-sulfophenyl-3,5-dicarbomethoxybenzene, 6-sulfo-2-naphthyl-3,5-dicarbomethoxybenzene, sulfo-terephthalic acid, dimethyl-sulfo-terephthalate, 5-sulfo-isophthalic acid, dialkyl-sulfo-terephthalate, sulfo-p-hydroxybenzoic acid, N,N-bis(2-hydroxyethyl)-2-amino ethane sulfonate, or mixtures thereof. The polyacid may be selected in an amount of, for example, from about 40 to about 60 mole %, from about 42 to 52 mole %, from about 45 to about 50 mole % and optionally, a second polyacid can be selected in an amount from about 0.1 to about 10 mole % of the resin.

Specific crystalline resins include poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), poly(decylene-sebacate), poly(decylene-decanoate), poly(ethylene-decanoate), poly(ethylene-dodecanoate), poly(nonylene-sebacate), poly(nonylene-decanoate), copoly(ethylene-fumarate)-copoly(ethylene-secate), copoly(ethylene-fumarate)-copoly(ethylene-decanoate), copoly(ethylene-fumarate)-copoly(ethylene-dodecanoate), copoly(2,2-dimethylpropane-1,3-diol-decanoate)-copoly(ethylene-adipate), alkali copoly(5-sulfoisophthaloyl)-copoly(propylene-adipate), alkali copoly(5-sulfoisophthaloyl)-copoly(butylene-adipate), alkali

copoly(5-sulfo-isophthaloyl)-copoly(pentylene-adipate), alkali copoly(5-sulfo-isophthaloyl)-copoly(hexylene-adipate), alkali copoly(5-sulfo-isophthaloyl)-copoly(octylene-adipate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(octylene-adipate), alkali copoly(5-sulfoisophthaloyl)-copoly(ethylene-succinate), alkali copoly(5-sulfoisophthaloyl)-copoly(propylene-succinate), alkali copoly(5-sulfoisophthaloyl)-copoly(butylene-succinate), alkali copoly(5-sulfoisophthaloyl)-copoly(pentylene-succinate), alkali copoly(5-sulfoisophthaloyl)-copoly(ethylene-succinate), alkali copoly(5-sulfoisophthaloyl)-copoly(hexylene-succinate), alkali copoly(5-sulfoisophthaloyl)-copoly(ethylene-sebacate), alkali copoly(5-sulfo-isophthaloyl)-copoly(propylene-sebacate), alkali copoly(5-sulfo-isophthaloyl)-copoly(butylene-sebacate), alkali copoly(5-sulfo-isophthaloyl)-copoly(pentylene-sebacate), alkali copoly(5-sulfo-isophthaloyl)-copoly(ethylene-sebacate), alkali copoly(5-sulfo-isophthaloyl)-copoly(hexylene-sebacate), alkali copoly(5-sulfo-isophthaloyl)-copoly(octylene-sebacate), alkali copoly(5-sulfo-isophthaloyl)-copoly(ethylene-adipate), alkali copoly(5-sulfo-isophthaloyl)-copoly(propylene-adipate), alkali copoly(5-sulfo-isophthaloyl)-copoly(butylene-adipate), alkali copoly(5-sulfo-isophthaloyl)-copoly(pentylene-adipate), alkali copoly(5-sulfo-isophthaloyl)-copoly(hexylene-adipatenonylene-decanoate), poly(octylene-adipate), and so on, wherein alkali is a metal like sodium, lithium or potassium. Examples of polyamides include poly(ethylene-adipamide), poly(propylene-adipamide), poly(butylene-adipamide), poly(pentylene-adipamide), poly(hexylene-adipamide), poly(octylene-adipamide), poly(ethylene-succinimide), and poly(propylene-sebecamide). Examples of polyimides include poly(ethylene-adipimide), poly(propylene-adipimide), poly(butylene-adipimide), poly(pentylene-adipimide), poly(hexylene-adipimide), poly(octylene-adipimide), poly(ethylene-succinimide), poly(propylene-succinimide), and poly(butylene-succinimide).

Suitable crystalline resins which may be utilized, optionally in combination with an amorphous resin as described above, include those disclosed in U.S. Pub. No 2006/0222991, the disclosure of which is hereby incorporated by reference in entirely.

In embodiments, a suitable crystalline resin may include a resin formed of ethylene glycol and a mixture of dodecanedioic acid and fumaric acid co-monomers.

The crystalline resin may be present, for example, in an amount from about 1 to about 85% by weight of the toner components, from about 2 to about 50% by weight, from about 5 to about 35% by weight of the toner components. The crystalline resin can possess various melting points of, for example, from about 30° C. to about 120° C., from about 50° C. to about 90° C., from about 60° C. to about 80° C. The crystalline resin may have a number average molecular weight ( $M_n$ ), as measured by gel permeation chromatography (GPC) of, for example, from about 1,000 to about 50,000, from about 2,000 to about 25,000, and a weight average molecular weight ( $M_w$ ) of, for example, from about 2,000 to about 100,000, from about 3,000 to about 80,000, as determined by GPC. The molecular weight distribution ( $M_w/M_n$ ) of the crystalline resin may be, for example, from about 2 to about 6, from about 3 to about 4.

## b. Crosslinking

Branching agents can be used and include, for example, a multivalent polyacid such as 1,2,4-benzene-tricarboxylic acid, 1,2,4-cyclohexanetricarboxylic acid, 2,5,7-naphthalenetricarboxylic acid 1,2,4-naphthalenetricarboxylic acid, 1,2,5-hexanetricarboxylic acid, 1,3-dicarboxyl-2-methyl-2-methylene-carboxylpropane, tetra(methylene-carboxyl) methane, 1,2,7,8-octanetetracarboxylic acid, acid anhydrides thereof, lower alkyl esters thereof and so on. The branching agent can be used in an amount from about 0.01 to about 10 mole % of the resin, from about 0.05 to about 8 mole % or from about 0.1 to about 5 mole % of the resin.

It may be desirable to crosslink the polymer. A suitable resin conducive to crosslinking is one with a reactive group, such as, a C=C bond or with pendant or side groups, such as, a carboxylic acid group. The resin can be crosslinked, for example, through free radical polymerization with an initiator. Suitable initiators include peroxides such as, organic peroxides or azo compounds, for example diacyl peroxides, such as, decanoyl peroxide, lauroyl peroxide and benzoyl peroxide, ketone peroxides, such as cyclohexanone peroxide and methyl ethyl ketone, alkyl peroxy esters, such as, t-butyl peroxy neodecanoate, 2,5-dimethyl 2,5-di(2-ethyl hexanoyl peroxy) hexane, t-amyl peroxy 2-ethyl hexanoate, t-butyl peroxy 2-ethyl hexanoate, t-butyl peroxy acetate, t-amyl peroxy acetate, t-butyl peroxy benzoate, t-amyl peroxy benzoate, alkyl peroxides, such as, dicumyl peroxide, 2,5-dimethyl 2,5-di(t-butyl peroxy)hexane, t-butyl cumyl peroxide, bis(t-butyl peroxy)diisopropyl benzene di-t-butyl peroxide and 2,5-dimethyl 2,5-di(t-butyl peroxy)hexyne-3, alkyl hydroperoxides, such as, 2,5-dihydro peroxy 2,5-dimethyl hexane, cumene hydroperoxide, t-butyl hydroperoxide and t-amyl hydroperoxide, and alkyl peroxyketals, such as, n-butyl 4,4-di(t-butyl peroxy)valerate, 1,1-di(t-butyl peroxy)3,3,5-trimethyl cyclohexane, 1,1-di(t-butyl peroxy)cyclohexane, 1,1-di(t-amyl peroxy)cyclohexane, 2,2-di(t-butyl peroxy)butane, ethyl 3,3-di(t-butyl peroxy)butyrate and ethyl 3,3-di(t-amyl peroxy)butyrate, azobis-isobutyronitrile, 2,2'-azobis(isobutyronitrile), 2,2'-azobis(2,4-dimethyl valeronitrile), 2,2'-azobis (methyl butyronitrile), 1,1'-azobis(cyano cyclohexane), 1,1-di(t-butyl peroxy)-3,3,5-trimethylcyclohexane, combinations thereof and the like. The amount of initiator used is proportional to the degree of crosslinking, and thus, the gel content of the polyester material. The amount of initiator used may range from, for example, about 0.01 to about 10 weight %, or from about 0.1 to about 5 weight % of the polyester resin. In the crosslinking, it is desirable that substantially all of the initiator be consumed. The crosslinking may be carried out at high temperature, and thus the reaction may be rapid, for example, less than 10 minutes, such as from about 20 seconds to about 2 minutes residence time.

Generally, as known in the art, the polyacid/polyester and polyols reagents, are mixed together, optionally with a catalyst, and incubated at an elevated temperature, such as, from about 180° C. or more, from about 190° C. or more, from about 200° C. or more, and so on, which can be conducted anaerobically, to enable esterification to occur until equilibrium, which generally yields water or an alcohol, such as, methanol, arising from forming the ester bonds in esterification reactions. The reaction can be conducted under vacuum to promote polymerization.

Hence, disclosed herein is a polyester resin suitable for use in imaging which can comprise a mixture of the relevant reagents prior to polymerization, such as, a polyacid/polyester reagent, and a polyol reagent whether polymerized or not. In embodiments, a polyester resin is produced and processed to form a polymer reagent, which can be dried and formed

into flowable particles, such as, a pellet, a powder and the like. The polymer reagent then can be incorporated with, for example, other reagents suitable for making a toner particle, such as, a colorant and/or a wax, and processed in a known manner to produce toner particles.

Polyester resins suitable for use in an imaging device are those which carry one or more properties, such as, a  $T_g$  (onset) of at least about 40° C., at least about 45° C., at least about 50° C.; a  $T_g$  of at least about 100° C., at least about 105° C., at least about 110° C.; an acid value (AV) of at least about 5, at least about 7, at least about 9; and an  $M_w$  of at least about 5000, at least about 15,000, at least about 20,000.

## 2. Colorants

Suitable colorants include those comprising carbon black, such as, REGAL 330® and Nipex 35; magnetites, such as, Mobay magnetites, MO8029™ and MO8060™; Columbia magnetites, MAPICO® BLACK; surface-treated magnetites; Pfizer magnetites, CB4799™, CB5300™, CB5600™ and MCX6369™, Bayer magnetites, BAYFERROX 8600™ and 8610™, Northern Pigments magnetites, NP-604™ and NP-608™, Magnox magnetites, TMB-100™ or TMB-104™; and the like.

Colored pigments, such as cyan, magenta, yellow, red, orange, green, brown, blue or mixtures thereof can be used. The additional pigment or pigments can be used as water-based pigment dispersions.

Examples of pigments include HELIOGEN BLUE L6900™, D6840™, D7080™, D7020™, PYLAM OIL BLUE™, PYLAM OIL YELLOW™, and PIGMENT BLUE 1™ available from Paul Uhlich & Company, Inc.; PIGMENT VIOLET 1™, PIGMENT RED 48™, LEMON CHROME YELLOW DCC 1026™, TOLUIDINE RED™ and BON RED C™ available from Dominion Color Corporation, Ltd., Toronto, Ontario; NOVAPERM YELLOW FGL™ and HOS-TAPERM PINK E™ from Hoechst; CINQUASIA MAGENTA™ available from E.I. DuPont de Nemours & Co., and the like.

Examples of magenta pigments include 2,9-dimethyl-substituted quinacridone, an anthraquinone dye identified in the Color Index as CI 60710, CI Dispersed Red 15, a diazo dye identified in the Color Index as CI 26050, CI Solvent Red 19, pigment red (PR) 269 and the like.

Illustrative examples of cyan pigments include copper tetra(octadecylsulfonamido) phthalocyanine, a copper phthalocyanine pigment listed in the Color Index as CI 74160, CI Pigment Blue, Pigment Blue 15:3, Pigment Blue 15:4, an Anthraazine Blue identified in the Color Index as CI 69810, Special Blue X-2137 and the like.

Illustrative examples of yellow pigments are diarylide yellow 3,3-dichlorobenzidine acetoacetanilide, a monoazo pigment identified in the Color Index as CI 12700, CI Solvent Yellow 16, a nitrophenyl amine sulfonamide identified in the Color Index as Foron Yellow SE/GLN, CI Disperse Yellow 3,2,5-dimethoxy-4-sulfonanilide phenylazo-4'-chloro-2,5-dimethoxy acetoacetanilide and Permanent Yellow FGL.

Other known colorants can be used, such as Levanyl Black A-SF (Miles, Bayer) and Sunperse Carbon Black LHD 9303 (Sun Chemicals), and colored dyes, such as, Neopen Blue (BASF), Sudan Blue OS (BASF), PV Fast Blue B2G 01 (American Hoechst), Sunperse Blue BHD 6000 (Sun Chemicals), Irgalite Blue BCA (CibaGeigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen

Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), SUCD-Yellow D1355 (BASF), Hostaperm Pink E (American Hoechst), Fanal Pink D4830 (BASF), Cinquasia Magenta (DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Orcet Pink RF (Ciba-Geigy), Paliogen Red 3871K (BASF), Paliogen Red 3340 (BASF), Lithol Fast Scarlet L4300 (BASF), combinations of the foregoing and the like. Other pigments that can be used, and which are commercially available include various pigments in the color classes, Pigment Yellow 74, Pigment Yellow 14, Pigment Yellow 83, Pigment Orange 34, Pigment Red 238, Pigment Red 122, Pigment Red 48:1, Pigment Red 53:1, Pigment Red 57:1, Pigment Red 83:1, Pigment Violet 23, Pigment Green 7 and so on, and combinations thereof.

The colorant, for example carbon black, cyan, magenta and/or yellow colorant, may be incorporated in an amount sufficient to impart the desired color to the toner. In general, pigment or dye, may be employed in an amount ranging from about 1% to about 35% by weight of the toner particles on a solids basis, from about 2% to about 25% by weight, from about 3% to about 15% by weight.

In embodiments, more than one pigment may be present in a toner particle. For example, two colorants may be present in a toner particle, such as, a first colorant of pigment blue, may be present in an amount ranging from about 2% to about 10% by weight of the toner particle on a solid basis, from about 3% to about 8% by weight or from about 5% to about 10% by weight; with a second colorant of pigment yellow that may be present in an amount ranging from about 5% to about 20% by weight of a toner particle on a solid basis, from about 6% to about 15% by weight or from about 10% to about 20% by weight and so on.

The pigment particles are selected to comprise a BET surface area of from about 60 m<sup>2</sup>/g to about 62 m<sup>2</sup>/g, from about 70 m<sup>2</sup>/g to about 90 m<sup>2</sup>/g, from about 75 m<sup>2</sup>/g to about 85 m<sup>2</sup>/g.

### 3. Optional Components

#### a. Surfactants

In embodiments, toner compositions may be in dispersions including surfactants. Emulsion aggregation methods where the polymer and other components of the toner are in combination can employ one or more surfactants to form an emulsion.

One, two or more surfactants may be used. The surfactants may be selected from ionic surfactants and nonionic surfactants, or combinations thereof. Anionic surfactants and cationic surfactants are encompassed by the term, "ionic surfactants."

The surfactant or the total amount of surfactants may be used in an amount of from about 0.01% to about 5% by weight of the toner-forming composition, for example, from about 0.75% to about 4% by weight, from about 1% to about 3% by weight of the toner-forming composition.

Examples of nonionic surfactants include, for example, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether and dialkylphenoxy poly(ethylene-neoxy) ethanol, for example, available from Rhone-Poulenc

as IGEPAL CA-210<sup>TM</sup>, IGEPAL CA-520<sup>TM</sup>, IGEPAL CA-720<sup>TM</sup>, IGEPAL CO-890<sup>TM</sup>, IGEPAL CO-720<sup>TM</sup>, IGEPAL CO-290<sup>TM</sup>, IGEPAL CA-210<sup>TM</sup>, ANTAROX 890<sup>TM</sup> and ANTAROX 897<sup>TM</sup>. Other examples of suitable nonionic surfactants include a block copolymer of polyethylene oxide and polypropylene oxide, including those commercially available as SYNPERONIC<sup>®</sup> PR/F, SYNPERONIC<sup>®</sup> PR/F 108; and a DOWFAX, available from The Dow Chemical Corp.

10 Anionic surfactants include sulfates and sulfonates, such as, sodium dodecylsulfate (SDS), sodium dodecylbenzene sulfonate, sodium dodecylphthalene sulfate and so on; dialkyl benzenealkyl sulfates; acids, such as, palmitic acid, and NEOGEN or NEOGEN SC obtained from Daiichi Kogyo Seiyaku, and so on, combinations thereof and the like. Other suitable anionic surfactants include, in embodiments, alkyl-diphenyloxide disulfonates or TAYCA POWER BN2060 from Tayca Corporation (Japan), which is a branched sodium dodecyl benzene sulfonate. Combinations of those surfactants and any of the foregoing nonionic surfactants may be used in embodiments.

15 Examples of cationic surfactants include, for example, alkylbenzyl dimethyl ammonium chloride, dialkyl benzene-alkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, trimethyl ammonium bromides, halide salts of quarternized polyoxyethylalkylamines, dodecylbenzyl triethyl ammonium chlorides, MIRAPOL<sup>®</sup> and 20 ALKAQUAT<sup>®</sup> available from Alkaril Chemical Company, SANISOL<sup>®</sup> (benzalkonium chloride) available from Kao Chemicals and the like, and mixtures thereof, including, for example, a nonionic surfactant as known in the art or provided hereinabove.

#### b. Waxes

25 The toners of the instant disclosure, optionally, may contain a wax, which can be either a single type of wax or a mixture of two or more different types of waxes (hereinafter identified as, "wax"). A wax can be added to a toner formulation or to a developer formulation, for example, to improve particular toner properties, such as, toner particle shape, charging, fusing characteristics, gloss, stripping, offset properties and the like. Alternatively, a combination of waxes can be added to provide multiple properties to a toner or a developer composition. A wax may be included as, for example, a fuser roll release agent.

30 The wax may be combined with the resin-forming composition for forming toner particles. When included, the wax may be present in an amount of, for example, from about 1 wt % to about 25 wt % of the toner particles, from about 5 wt % to about 20 wt % of the toner particles.

35 Waxes that may be selected include waxes having, for example, a weight average molecular weight of from about 500 to about 20,000, from about 1,000 to about 10,000.

40 Waxes that may be used include, for example, polyolefins, such as, polyethylene, polypropylene and polybutene waxes, such as, those that are commercially available, for example, POLYWAX<sup>TM</sup> polyethylene waxes from Baker Petrolite, wax emulsions available from Michaelman, Inc. or Daniels Products Co., EPOLENE N15<sup>TM</sup> which is commercially available from Eastman Chemical Products, Inc., VISCOL 550-PT<sup>™</sup>, a low weight average molecular weight polypropylene available from Sanyo Kasei K.K.; plant-based waxes, such as carnauba wax, rice wax, candelilla wax, sumac wax and jojoba oil; animal-based waxes, such as beeswax; mineral-based waxes and petroleum-based waxes, such as montan wax, ozokerite, ceresin wax, paraffin wax, microcrystalline

## 11

wax and Fischer-Tropsch waxes; ester waxes obtained from higher fatty acids and higher alcohols, such as stearyl stearate and behenyl behenate; ester waxes obtained from higher fatty acids and monovalent or multivalent lower alcohols, such as butyl stearate, propyl oleate, glyceride monostearate, glyceride distearate and pentaerythritol tetrabehenate; ester waxes obtained from higher fatty acids and multivalent alcohol multimers, such as diethyleneglycol monostearate, dipropylene-glycol distearate, diglyceryl distearate and triglyceryl tetrastearate; sorbitan higher fatty acid ester waxes, such as sorbitan monostearate; cholesterol higher fatty acid ester waxes, such as, cholesteryl stearate, and so on.

Examples of functionalized waxes that may be used include, for example, amines and amides, for example, AQUA SUPERSLIP 6550<sup>TM</sup> and SUPERSLIP 6530<sup>TM</sup> available from Micro Powder Inc.; fluorinated waxes, for example, POLYFLUO 190<sup>TM</sup>, POLYFLUO 200<sup>TM</sup>, POLYSILK 19<sup>TM</sup> and POLYSILK 14<sup>TM</sup> available from Micro Power Inc.; mixed fluorinated amide waxes, for example, MICROSERSION 19<sup>TM</sup> also available from Micro Powder Inc.; imides, esters, quaternary amines, carboxylic acids, acrylic polymer emulsions, for example, JONCRYL 74<sup>TM</sup>, 89<sup>TM</sup>, 130<sup>TM</sup>, 537<sup>TM</sup> and 538<sup>TM</sup> available from SC Johnson Wax; and chlorinated polypropylenes and polyethylenes available from Allied Chemical, Petrolite Corp. and SC Johnson. Mixtures and combinations of the foregoing waxes also may be used in embodiments.

## c. Aggregating Factor

An aggregating factor may be used, and may be an inorganic cationic coagulant, such as, for example, polyaluminum chloride (PAC), polyaluminum sulfosilicate (PASS), aluminum sulfate, zinc sulfate, magnesium sulfate, chlorides of magnesium, calcium, zinc, beryllium, aluminum, sodium, other metal halides including monovalent and divalent halides.

The aggregating factor may be present in an emulsion in an amount of from, for example, from about 0 to about 10 wt %, from about 0.05 to about 5 wt % based on the total solids in the toner.

The aggregating factor may also contain minor amounts of other components, for example, nitric acid.

In embodiments, a sequestering agent or chelating agent may be introduced after aggregation is complete to adjust pH and/or to sequester or to extract a metal complexing ion, such as, aluminum from the aggregation process. Thus, the sequestering, chelating or complexing agent used after aggregation is complete may comprise an organic complexing component, such as, ethylenediaminetetraacetic acid (EDTA), gluconal, hydroxyl-2,2'iminodisuccinic acid (HIDS), dicarboxymethyl glutamic acid (GLDA), methyl glycidyl diacetic acid (MGDA), hydroxydiethyliminodiacetic acid (HIDA), sodium gluconate, potassium citrate, sodium citrate, nitrotriacetate salt, humic acid, fulvic acid; salts of EDTA, such as, alkali metal salts of EDTA, tartaric acid, gluconic acid, oxalic acid, polyacrylates, sugar acrylates, citric acid, polyaspartic acid, diethylenetriamine pentaacetate, 3-hydroxy-4-pyridinone, dopamine, eucalyptus, iminodisuccinic acid, ethylenediaminedisuccinate, polysaccharide, sodium ethylenedinitrilotetraacetate, thiamine pyrophosphate, farnesyl pyrophosphate, 2-aminoethylpyrophosphate, hydroxyl ethylen-1,1-diphosphonic acid, aminotrimethylenephosphonic acid, diethylene triaminepentamethylene phosphonic acid, ethylenediamine tetramethylene phosphonic acid, and mixtures thereof.

## d. Surface Additive

In embodiments, the toner particles can be mixed with one or more of silicon dioxide or silica (SiO<sub>2</sub>), titania or titanium

## 12

dioxide (TiO<sub>2</sub>) and/or cerium oxide. Silica may be a first silica and a second silica. The first silica may have an average primary particle size, measured in diameter, in the range of, for example, from about 5 nm to about 50 nm, from about 5 nm to about 25 nm, from about 20 nm to about 40 nm. The second silica may have an average primary particle size, measured in diameter, in the range of, for example, from about 100 nm to about 200 nm, from about 100 nm to about 150 nm, from about 125 nm to about 145 nm. The second silica may have a larger average size (diameter) than the first silica. The titania may have an average primary particle size in the range of, for example, about 5 nm to about 50 nm, from about 5 nm to about 20 nm, from about 10 nm to about 50 nm. The cerium oxide may have an average primary particle size in the range of, for example, about 5 nm to about 50 nm, from about 5 nm to about 20 nm, from about 10 nm to about 50 nm.

Zinc stearate also may be used as an external additive. Calcium stearate and magnesium stearate may provide similar functions. Zinc stearate may have an average primary particle size in the range of, for example, from about 500 nm to about 650 nm.

## B. Toner Particle Preparation

## 1. Method

## a. Particle Formation

The toner particles may be prepared by any method within the purview of one skilled in the art, for example, any of the emulsion/aggregation (EA) methods can be used with the polyester resin. However, any suitable method of preparing toner particles may be used, including chemical processes, such as, suspension and encapsulation processes disclosed, for example, in U.S. Pat. Nos. 5,290,654 and 5,302,486, the disclosures of each of which are hereby incorporated by reference in entirety; by conventional granulation methods, such as, jet milling; pelletizing slabs of material; other mechanical processes; any process for producing nanoparticles or micro-particles; and so on.

In embodiments relating to an emulsification/aggregation process, a resin can be dissolved in a solvent, and can be mixed into an emulsion medium, for example water, such as, deionized water, optionally containing a stabilizer, and optionally a surfactant. Examples of suitable stabilizers include water-soluble alkali metal hydroxides, such as, sodium hydroxide, potassium hydroxide, lithium hydroxide, beryllium hydroxide, magnesium hydroxide, calcium hydroxide or barium hydroxide; ammonium hydroxide; alkali metal carbonates, such as, sodium bicarbonate, lithium bicarbonate, potassium bicarbonate, lithium carbonate, potassium carbonate, sodium carbonate, beryllium carbonate, magnesium carbonate, calcium carbonate, barium carbonate or cesium carbonate, or mixtures thereof. When a stabilizer is used, the stabilizer can be present in amounts of from about 0.1% to about 5%, from about 0.5% to about 3% by weight of the resin. The stabilizer can be added to the mixture at ambient temperature, or can be heated to the mixture temperature prior to addition.

Following emulsification, toner compositions may be prepared by aggregating a mixture of one or more resins, one or more pigments, an optional wax and any other desired additives in an emulsion, optionally, with surfactants as described above, and then optionally coalescing the aggregate mixture. A mixture may be prepared by adding an optional wax or other materials, which may also be optionally in a dispersion, including a surfactant, to the emulsion comprising a resin-forming material and a pigments, which may be a mixture of two or more emulsions containing the requisite reagents. The pH of the resulting mixture may be adjusted with an acid,

## 13

such as, for example, acetic acid, nitric acid or the like. In embodiments, the pH of the mixture may be adjusted to from about 2 to about 4.5.

Additionally, in embodiments, the mixture may be homogenized. If the mixture is homogenized, mixing can be at from about 600 to about 4,000 rpm. Homogenization may be by any suitable means, including, for example, an IKA ULTRA TURRAX T50 probe homogenizer.

## b. Aggregation

Following preparation of the above mixture, often, it is desirable to form larger particles or aggregates, often sized in micrometers, of the smaller particles from the initial polymerization reaction, often size in nanometers. An aggregating factor (or coagulant) may be added to the mixture. Suitable aggregating factors include, for example, aqueous solutions of a divalent cation, a multivalent cation or a compound comprising same.

In embodiments, the aggregating factor may be added to the mixture at a temperature that is below the glass transition temperature ( $T_g$ ) of the resin or of a polymer.

The aggregating factor may be added to the mixture in an amount of, for example, from about 0.1 part per hundred (pph) to about 5 pph, from about 0.2 pph to about 2 pph of the reaction mixture.

To control aggregation, the aggregating factor may be metered into the mixture over time. For example, the factor may be added incrementally from about 5 to about 240 minutes, from about 30 to about 200 minutes.

Addition of the aggregating factor may be done while the mixture is homogenized. If the mixture is homogenized, mixing can be at from about 600 to about 4,000 rpm. Homogenization may be by any suitable means, including, for example, an IKA ULTRA TURRAX T50 probe homogenizer, and at a temperature that is below the  $T_g$  of the resin or polymer, from about 0° C. to about 60° C., from about 1° C. to about 50° C. The growth and shaping of the particles following addition of the aggregation factor may be accomplished under any suitable condition(s).

Addition of the aggregating factor also may be done while the mixture is maintained under stirred conditions, from about 50 rpm to about 1,000 rpm, from about 100 rpm to about 500 rpm.

The particles may be permitted to aggregate until a predetermined desired particle size is obtained. Particle size can be monitored during the growth process. For example, samples may be taken during the growth process and analyzed, for example, with a COULTER COUNTER, for average particle size. The aggregation thus may proceed by maintaining the mixture, for example, at elevated temperature, or slowly raising the temperature, for example, from about 40° C. to about 100° C., and holding the mixture at that temperature for from about 0.5 hours to about 6 hours, from about hour 1 to about 5 hours, while maintaining stirring, to provide the desired aggregated particles. Once the predetermined desired particle size is attained, the growth process is halted.

Once the desired final size of the toner particles or aggregates is achieved, the pH of the mixture may be adjusted with base to a value of from about 5 to about 12, from about 6 to about 10. The adjustment of pH may be used to freeze, that is, to stop, toner particle growth. The base used to stop toner particle growth may be, for example, an alkali metal hydroxide, such as, for example, sodium hydroxide, potassium hydroxide, ammonium hydroxide, combinations thereof and the like. In embodiments, a chelator, such as, EDTA, may be added to assist adjusting the pH to the desired value.

The characteristics of the toner particles may be determined by any suitable technique and apparatus. Volume aver-

## 14

age particle diameter and geometric standard deviation may be measured using an instrument, such as, a Beckman Coulter MULTISIZER 3, operated in accordance with the instructions of the manufacturer.

5 The aggregated particles may be of a size of about 4  $\mu\text{m}$  or more, for example, at least the 5.53  $\mu\text{m}$ , at least about 5.55  $\mu\text{m}$ , at least about 5.57  $\mu\text{m}$  in  $D_{50}$  volume diameter.

## c. Shells

10 In embodiments, an optional shell may be applied to the formed toner particles, aggregates or coalesced particles. Any polymer, including those described above as suitable for the core, may be used for the shell. The shell polymer may be applied to the particles or aggregates by any method within the purview of those skilled in the art.

15 In embodiments, an amorphous polyester resin may be used to form a shell over the particles or aggregates to form toner particles or aggregates having a core-shell configuration. In some embodiments, a low molecular weight amorphous polyester resin may be used to form a shell over the particles or aggregates.

Formation of the shell over the aggregated particles may occur while heating to a temperature from about 30° C. to about 80° C., from about 35° C. to about 70° C. The formation of the shell may take place for a period of time from about 5 minutes to about 10 hours, from about 10 minutes to about 5 hours.

20 The shell polymer may be present in an amount of from about 1% to about 80% by weight of the toner panicles or aggregates, from about 5% to about 50% by weight of the toner particles or aggregates.

## d. Coalescence

25 Following aggregation to a desired particle size and application of any optional shell, the particles then may be coalesced to a desired final shape, such as, a circular shape, for example, to correct for irregularities in shape and size, the coalescence being achieved by, for example, heating the mixture to a temperature from about 45° C. to about 100° C., from about 55° C. to about 99° C. which may be at or above the  $T_g$  of the resins used to form the toner panicles, and/or reducing the stirring, for example, to from about 1000 to about 100 rpm, from about 800 rpm to about 200 rpm. Coalescence may be conducted over a period front about 0.01 to about 9 hours, 30 irons about 0.1 to about 4 hours, see, for example, U.S. Pat. No. 7,710,831.

35 Alter aggregation and/or coalescence, the mixture may be cooled to room temperature, such as, from about 20° C. to about 25° C. The cooling may be rapid or slow, as desired. A suitable cooling method may include introducing cold water to a jacket around the reactor or discharging toner into cold water. After cooling, the toner panicles optionally may be washed with water and then dried. Drying may be by any suitable method, including, for example, freeze-drying.

40 Optionally, a coalescing agent can be used. Examples of suitable coalescence agents include, but are not limited to, benzoic acid alkyl esters, ester alcohols, glycol/ether-type solvents, long chain aliphatic alcohols, aromatic alcohols, mixtures thereof and the like.

45 In embodiments, the coalescence agent (or coalescing agent or coalescence aid agent) evaporates during later stages of the emulsion/aggregation process, such as, during a second heating step, that is, generally above the  $T_g$  of the resin or a polymer. The final toner particles are thus, free of, or essentially or substantially free of any remaining coalescence agent. To the extant that any remaining coalescence agent may be present in a final toner particle, the amount of remain-

## 15

ing coalescence agent is such that presence thereof does not affect any properties or the performance of the toner or developer.

The coalescence agent can be added prior to the coalescence or fusing step in any desired or suitable amount. For example, the coalescence agent can be added in an amount of from about 0.01 to about 10% by weight, based on the solids content in the reaction medium, or from about 0.05, or from about 0.1%, to about 0.5 or to about 3.0% by weight, based on the solids content in the reaction medium. Of course, amounts outside those ranges can be used, as desired.

In embodiments, the coalescence agent can be added at any time between aggregation and coalescence, although in some embodiments it may be desirable to add the coalescence agent after aggregation is, "frozen," or completed, for example, by adjustment of pH, for example, by addition, for example, of base.

## e. Optional Additives

In embodiments, the toner particles also may contain other optional additives.

## i. Charge Additives

The toner may include any known charge additives in amounts of from about 0.1 to about 10 weight %, of from about 0.5 to about 7 weight % of the toner. Examples of such charge additives include alkyl pyridinium halides, bisulfates, the charge control additives of U.S. Pat. Nos. 3,944,493; 4,007,293; 4,079,014; 4,394,430; and 4,560,635, the disclosures of each of which are hereby incorporated by reference in entirety, negative charge enhancing additives, such as, aluminum complexes, and the like.

Charge enhancing molecules can be used to impart either a positive or negative charge on a toner particle. Examples include quaternary ammonium compounds, see, for example, U.S. Pat. No. 4,298,672, organic sulfate and sulfonate compounds, see for example, U.S. Pat. No. 4,338,390, cetyl pyridinium tetrafluoroborates, distearyl dimethyl ammonium methyl sulfate, aluminum salts and so on.

Such enhancing molecules can be present in an amount of from about 0.1 to about 10% or from about 1 to about 3% by weight.

## ii. Surface Modifications

Surface additives can be added to the toner compositions of the present disclosure, for example, after washing or drying. Examples of such surface additives include, for example, one or more of a metal salt a metal salt of a fatty acid, a colloidal silica, a metal oxide such as,  $TiO_2$  (for example, for improved RH stability, tribo control and improved development and transfer stability), an aluminum oxide, a cerium oxide, a strontium titanate,  $SiO_2$ , mixtures thereof and the like. Examples of such additives include those disclosed in U.S. Pat. Nos. 3,590,000; 3,720,617; 3,655,374; and 3,983,045, the disclosures of each of which are hereby incorporated by reference in entirety.

Surface additives may be used in an amount of from about 0.1 to about 10 wt % or front about 0.5 to about 7 wt % of the toner.

Other surface additives include lubricants, such as, a metal salt of a fatty acid (e.g., zinc or calcium stearate) or long chain alcohols, such as, UNILIN 700 available from Baker Petrolite and AEROSIL R972® available from Degussa. The coated silicas of U.S. Pat. Nos. 6,190,815 and 6,004,714, the disclosures of each of which hereby are incorporated by reference in entirety, also can be present. The additive can be present in an amount of from about 0.05 to about 5%, front about 0.1 to about 2% of the toner, which additives can be added during the aggregation or blended into the formed toner product.

## 16

Silica, for example, can enhance toner flow, tribo control, admix control, improved development and transfer stability and higher toner blocking temperature. Zinc, calcium or magnesium stearate also can provide developer conductivity, tribo enhancement, higher toner charge and charge stability. The external surface additives can be used with or without a coating or shell.

The gloss of a toner may be influenced by the amount of retained metal ion, such as  $Al^{3+}$ , in a particle. The amount of retained metal ion may be adjusted further by the addition of a chelator, such as, EDTA. In embodiments, the amount of retained metal ion, for example,  $Al^{3+}$ , in toner particles of the present disclosure may be from about 0.1 pph to about 1 pph, from about 0.25 pph to about 0.8 pph. The gloss level of a toner of the instant disclosure may have a gloss, as measured by Gardner Gloss Units (gu), of from about 5 gu to about 100 gu, from about 10 gu to about 95 gu, from about 20 gu to about 90 gu.

Hence, a particle can contain at the surface one or more silicas, one or more metal oxides, such as, a titanium oxide and a cerium oxide, a lubricant, such as, a zinc stearate and so on. In embodiments, a particle surface can comprise two silicas, two metal oxides, such as, titanium oxide and cerium oxide, and a lubricant, such as, a zinc stearate. All of those surface components can comprise about 5% by weight of a toner particle weight. There can also be blended with the toner compositions, external additive particles including flow aid additives, which additives may be present on the surface of the toner particles. Examples of these additives include metal oxides like titanium oxide, tin oxide, mixtures thereof, and the like; colloidal silicas, such as AEROSIL®, metal salts and metal salts of fatty acids, including zinc stearate, aluminum oxides, cerium oxides, and mixtures thereof. Each of the external additives may be presented in amounts of from about 0.1 to about 5 wt %, from about 0.1 to about 1 wt %, of the toner. Several of the aforementioned additives are illustrated in U.S. Pat. Nos. 3,590,000, 3,800,588, and 6,214,507, the disclosures which are incorporated herein by reference.

Toners may possess suitable charge characteristics when exposed to extreme relative humidity (RH) conditions. The low humidity zone (C zone) may be about 10° C. and 15% RH, while the high humidity zone (A zone) may be about 28° C. and 85% RH.

Toners of the instant disclosure also may possess a parent toner charge per mass ratio (q/m) of from about  $-5 \mu C/g$  to about  $-90 \mu C/g$ , and a final toner charge after surface additive blending of from about  $-15 \mu C/g$  to about  $-80 \mu C/g$ .

Other desirable characteristics of a toner include storage stability, particle size integrity, high rate of fusing to the substrate or receiving member, sufficient release of the image from the photoreceptor, nondocument offset, use of smaller-size particles and so on, and such characteristics can be obtained by including suitable reagents, suitable additives or both, and/or preparing the toner with particular protocols.

The dry toner particles, exclusive of external surface additives, may have the following characteristics: (1) volume average diameter (also referred to as "volume average particle diameter") of at least about 5.53  $\mu m$ , at least about 5.5  $\mu m$ , at least about 5.57  $\mu m$ ; (2) number average geometric standard deviation (GSDn) and/or volume average geometric standard deviation (GSDv) of from about 1.18 to about 1.30, from about 1.21 to about 1.24; and (3) circularity from about 0.9 to about 1.0 (measured with, for example, a Sysmex FPIA 2100), from about 0.95 to about 0.985, from about 0.96 to about 0.98.

## II. Developers

## A. Composition

The toner particles thus formed may be formulated into a developer composition. For example, the toner particles may be mixed with carrier particles to achieve a two component developer composition. The toner concentration in the developer may be from about 1% to about 25% by weight of the total weight of the developer, from about 2% to about 15% by weight of the total weight of the developer, with the remainder of the developer composition being the carrier. However, different toner and carrier percentages may be used to achieve a developer composition with desired characteristics.

## 1. Carrier

Examples of carrier particles for mixing with the toner particles include those particles that are capable of triboelectrically obtaining a charge of polarity opposite to that of the toner particles. Illustrative examples of suitable carrier particles include granular zircon, granular silicon, glass, steel, nickel, ferrites, iron ferrites, silicon dioxide, one or more polymers and the like. Other carriers include those disclosed in U.S. Pat. Nos. 3,847,604; 4,937,166; and 4,935,326.

The carrier particles may include a core with a coating thereover, which may be formed from a polymer or a mixture of polymers that are not in close proximity thereto in the triboelectric series, such as, those as taught herein or as known in the art. The coating may include fluoropolymers, such as polyvinylidene fluorides, terpolymers of styrene, methyl methacrylates, silanes, such as triethoxy silanes, tetrafluoroethylenes, other known coatings and the like. For example, coatings containing polyvinylidenefluoride, available, for example, as KYNAR 301F™, and/or polymethyl-methacrylate (PMMA), for example, having a weight average molecular weight of about 300,000 to about 350,000, such as, commercially available from Soken, may be used. PMMA and polyvinylidenefluoride may be mixed in proportions of from about 30 to about 70 wt % to about 70 to about 30 wt %, from about 40 to about 60 wt % to about 60 to about 40 wt %. The coating may have a weight of from about 0.1 to about 5% by weight of the carrier, from about 0.5 to about 3% by weight of the carrier.

In embodiments, PMMA, for example, may be copolymerized with any desired monomer, so long as the resulting copolymer retains a suitable particle size. Suitable monomers include monoalkyl or dialkyl amines, such as, a dimethylaminoethyl methacrylate, diethylaminoethyl methacrylate, diisopropylaminoethyl methacrylate or butylaminoethyl methacrylate, and the like.

Various effective suitable means can be used to apply the polymer to the surface of the carrier core, for example, cascade roll mixing, tumbling, milling, shaking, electrostatic powder cloud spraying, fluidized bed mixing, electrostatic disc processing, electrostatic curtain processing, combinations thereof and the like. The mixture of carrier core particles and polymer then may be heated to enable the polymer to melt and to fuse to the carrier core. The coated carrier particles then may be cooled and thereafter classified to a desired particle size.

The carrier particles may be prepared by mixing the carrier core with polymer in an amount from about 0.05 to about 10% by weight, from about 0.01 to about 3% by weight, based on the weight of the coated carrier particle, until adherence thereof to the carrier core is obtained, for example, by mechanical impaction and/or electrostatic attraction.

In embodiments, suitable carriers may include a steel core, for example, of from about 25 to about 100  $\mu\text{m}$  in size, from about 50 to about 75  $\mu\text{m}$  in size, coated with about 0.5% by weight of a polymer mixture including, for example, methyl-

acrylate and carbon black, using the process described, for example, in U.S. Pat. Nos. 5,236,629 and 5,330,874.

## III. Devices Comprising a Toner Particle

Toners and developers can be combined with a number of devices ranging from enclosures or vessels, such as, a vial, a bottle, a flexible container, such as a bag or a package, and so on, to devices that serve more than a storage function.

## A. Imaging Device Components

The toner compositions and developers of interest can be incorporated into devices dedicated, for example, to delivering same for a purpose, such as, forming an image. Hence, particularized toner delivery devices are known, see, for example, U.S. Pat. No. 7,822,370, and can contain a toner preparation or developer of interest. Such devices include cartridges, tanks, reservoirs and the like, and can be replaceable, disposable or reusable. Such a device can comprise a storage portion; a dispensing or delivery portion; and so on; along with various ports or openings to enable toner or developer addition to and removal from the device; an optional portion for monitoring amount of toner or developer in the device; formed or shaped portions to enable siting and seating of the device in, for example, an imaging device; and so on.

## B. Toner or Developer Delivery Device

A toner or developer of interest may be included in a device dedicated to delivery thereof, for example, for recharging or refilling toner or developer in an imaging device component, such as, a cartridge, in need of toner or developer, see, for example, U.S. Pat. No. 7,817,944, wherein the imaging device component may be replaceable or reusable.

## IV. Imaging Devices

The toners or developers can be used for electrostaticographic or electrophotographic processes, including those disclosed in U.S. Pat. No. 4,295,990, the disclosure of which hereby is incorporated by reference in entirety. In embodiments, any known type of image development system may be used in an image developing device, including, for example, magnetic brush development, jumping single component development, hybrid scavengerless development (HSD) and the like. Those and similar development systems are within the purview of those skilled in the art.

Imaging processes include, for example, preparing an image with an electrophotographic device including, for example, one or more of a charging component, an imaging component, a photoconductive component, a developing component, a transfer component, a fusing component and so on. The electrophotographic device may include a high speed printer, a color printer and the like.

Once the image is formed with toners/developers via a suitable image development method, such as any of the aforementioned methods, the image then may be transferred to an image receiving medium or substrate, such as, a paper and the like. In embodiments, the fusing member or component, which can be of any desired or suitable configuration, such as, a drum or roller, a belt or web, a flat surface or platen, or the like, may be used to set the toner image on the substrate. Optionally, a layer of a liquid, such as, a fuser oil can be applied to the fuser member prior to fusion.

Color printers commonly use four housings carrying different colors to generate full color images based on black plus the standard printing colors, cyan, magenta and yellow. However, in embodiments, additional housings may be desirable, including image generating devices possessing five housings, six housings or more, thereby providing the ability to carry additional toner colors to print an extended range of colors (extended gamut).

The follow Examples illustrate embodiments of the instant disclosure. The Examples are intended to be illustrative only

and are not intended to limit the scope of the present disclosure. Parts and percentages are by weight unless otherwise indicated. As use herein, "room temperature," (RT) refers to a temperature of from about 20° C. to about 30° C.

## EXAMPLES

## Example 1

## EA Toner

A polyester EA toner was prepared at the 2 L bench scale comprising between 80-85 wt % amorphous, (DOWFAX® 2A1, Dow Chemical Company), 5-10 wt % wax ( $T_m=90^\circ\text{C}$ ), The International Group, Inc. (IGI), 4-7 wt % pigment and 1-2 wt % external additives, such as, silica or titanium oxide were mixed in a reactor. The slurry was homogenized and coagulant was mixed for aggregating the particles. The particles continued to aggregate to achieve the targeted particle size. Once at the target particle size, the pH was adjusted using sodium hydroxide (NaOH) and EDTA to raise the pH and to freeze particle growth. The process proceeded with an increase in reactor temperature and a pH adjustment to about using a pH 5.7 sodium acetate/acetic acid buffer where the particles coalesced. After about two hours of heating to coalesce the particles, a circularity  $>0.965$  was achieved and the particles were quench cooled with ice.

Toners were prepared with different pigments and the resulting toners were assessed for J zone performance. As an example, various samples of PR 269 were testing in a magenta toner. The pigment was obtained from Sanyo Color Works of Sun Chemical. The results are presented in the following table with a subject categorization of J zone performance.

TABLE 1

| Dry Pigment | Vol. Diameter<br>( $D_{50}$ $\mu\text{m}$ ) | BET (m <sup>2</sup> /g) | J Zone<br>Performance |
|-------------|---------------------------------------------|-------------------------|-----------------------|
| Sanyo       |                                             | 80                      | Good                  |
| Sun 1       |                                             | 73                      | Good                  |
| Sun 2       | 5.51                                        | 80                      | Good                  |
| Sun 3       | 5.46                                        | 96                      | Poor                  |
| Sun 4       |                                             | 102                     | Poor                  |
| Sun 5       |                                             | 105                     | Poor                  |
| Sun 6       | 5.29                                        | 125                     | Worst                 |
| Sun 7       |                                             | 129                     | Worst                 |
| Sun 8       | 5.57                                        | 84                      | Good                  |

It can be seen that PR 269 pigment particles with a BET of less than 96 m<sup>2</sup>/g have good toner performance. Generally particle size and surface area are related inversely. BET surface area can be a more exacting metric. Overall toner particle size has an effect, toner particles having a size greater than about 5.53  $\mu\text{m}$  also provide good performance.

It will be appreciated that various of the above-disclosed and other features and functions, or alternatives thereof, may be desirably combined into many other difference systems or applications. Also various presently unforeseen or unanticipated alternatives, modifications, variations or improvements therein may be subsequently made by those skilled in the art, which are also intended to be encompassed by the following claims. Unless specifically recited in a claim, steps or components of claims should not be implied or imported from the specification or any other claims as to any particular order, number, position, size, shape, angle, color or material.

All references cited herein are incorporated by reference in entirety.

We claim:

- Emulsion aggregation toner particles comprising a BET surface area from about 75 m<sup>2</sup>/g to about 85 m<sup>2</sup>/g, wherein circularity of said toner particles is between about 0.9 and about 1.0, and said toner particles comprise improved J zone charge.
- The toner particles of claim 1, wherein volume diameter of said toner particles is at least about 5.53  $\mu\text{m}$ .
- The toner particles of claim 1, wherein volume diameter of said toner particles is at least about 5.55  $\mu\text{m}$ .
- The toner particles of claim 1, comprising a polyacrylate resin.
- The toner particles of claim 1, comprising a polystyrene resin.
- The toner particles of claim 1, comprising an amorphous resin, a crystalline resin or both.
- The toner particles of claim 1, comprising a polyester resin.
- The toner particles of claim 1, comprising a wax.
- The toner particles of claim 1, comprising a shell.
- The toner particles of claim 1, comprising a second colorant.
- The toner particles of claim 1, wherein said magenta colorant comprises 2,9-dimethyl-substituted quinacridone, CI 60710, CI Dispersed Red 15, CI 26050, CI Solvent Red 19 or PR 269.
- The toner particles of claim 1 comprising from about 3 to about 15 wt % colorant.
- The toner particles of claim 1, comprising from about 2 to about 35 wt % colorant.
- The toner particles of claim 1 comprising a low melt toner.
- The toner particles of claim 1, comprising a charge control agent.
- The toner particles of claim 1, comprising a flow aid.
- The toner particles of claim 1, comprising a silica.
- The toner particles of claim 1, comprising a metal oxide.
- A developer comprising the toner particles of claim 1.
- The developer of claim 19 comprising a carrier.

\* \* \* \* \*